

# UNITED STATES PATENT OFFICE.

OSCAR JAECK, OF ELBERFELD, GERMANY, ASSIGNOR TO FARBENFABRIKEN OF ELBERFELD CO., OF NEW YORK, N. Y., A CORPORATION OF NEW YORK.

## PROCESS OF DYEING.

SPECIFICATION forming part of Letters Patent No. 717,749, dated January 6, 1903.

Application filed October 2, 1902. Serial No. 125,696. (No specimens.)

*To all whom it may concern:*

Be it known that I, OSCAR JAECK, doctor of philosophy, chemist, (assignor to the FARBENFABRIKEN OF ELBERFELD CO., of New York,) 5 residing at Elberfeld, Germany, have invented a new and useful Improvement in Processes of Dyeing; and I hereby declare the following to be a clear and exact description of my invention.

As is known, cotton goods dyed with sulfurized substantive coloring-matters are often subjected to an after-treatment for the purpose of rendering the shades faster or brighter. The steaming operation and the treatment 15 with hydrogen peroxid, with chromates, with sulfate of copper, with zinc salts, or the like are well-known operations. Another process of after-treatment was described in the United States Letters Patent No. 688,999, dated De- 20 cember 17, 1901. This process consists in treating cotton dyed with sulfurized dyestuffs with alkylating agents.

I have now found a new and valuable process of after-treatment, consisting in treating 25 the goods dyed with sulfurized dyestuffs with neutral sulfites, after which treatment it is suitable to expose them to the influence of the air. The results are remarkable, especially when using those dyestuffs which by the known 30 process of after-treatment give a still more valuable shade—such, for instance, as immedial blue C R, katigen-indigo B extra and R extra, immedial black V extra, katigen blue-black R, or the like. The action of the sul- 35 fites takes place with great facility. It is generally completed in a short time on working at a temperature of from 60° to 80° centigrade. The resulting shades are mostly distinguished for great brightness and fastness. They have 40 generally a certain resemblance to the shades obtained by steaming the dyed cotton in the presence of alkalies. The low price of the sulfites and the simple management are of great technical value for the new process of 45 after-treatment.

In carrying out my process practically I can

proceed as follows: The cotton, dyed with ten per cent. of immedial blue C R, rinsed, and exposed to the air for a short while, is placed in a bath containing two grams per liter of 50 neutral sodium sulfite. It is handled in the dye-bath for half an hour, (the temperature thereof being kept at about 80° centigrade,) rinsed, and dried. By means of this treatment the greenish-black shade of the cotton 55 turns into a bright navy-blue.

The process of after-treatment can also be carried out in the following manner: The dyed goods are rinsed and passed two or three times through a bath containing from one to 60 two per cent. of sodium sulfite, ( $Na_2SO_3$ ) The cotton is then squeezed and dried without further rinsing. By means of this operation the shade is changed in a manner similar to that above described. 65

It may, however, be pointed out that the temperature, the duration of after-treatment, and the quantities of sulfites can be varied within wide limits. On using higher temperatures and larger quantities of sulfites the 70 after-treatment is effected in a shorter time.

The process of after-treatment is the same when other sulfurized colors are used.

The same dyestuffs dyed on other fibers—for instance, on silk—give analogous results. 75

In the following table the change of shade of some sulfurized dyestuffs of commerce is indicated.

| Dyestuffs.              | Shade after dyeing.               | Shade after the treatment with sulfite. | 80 |
|-------------------------|-----------------------------------|-----------------------------------------|----|
| Katigen-black S W       | Jet black having a greenish tint. | Bluish black.                           |    |
| Katigen-indigo B extra. | Dull greenish black.              | Bright reddish blue.                    | 85 |
| Katigen-indigo R extra. | Dull reddish blue.                | Bright reddish blue.                    |    |
| Immedial black V extra. | Greenish black.                   | Dark blue.                              |    |
| Pyrogen-blue R.         | Greenish blue-black.              | Navy-blue.                              |    |
| Immedial blue C R.      | Greenish blue-black.              | Navy-blue.                              |    |
| Katigen blue-black R.   | Greenish black.                   | Dark navy-blue.                         |    |
| Katigen blue-black 4 B. | Greenish black.                   | Dark blue.                              |    |
| Pyrogen-black           | Greenish black.                   | Dark blue.                              | 90 |

Having now described my invention and in

what manner the same is to be performed, what I claim as new, and desire to secure by Letters Patent, is—

The herein-described process for producing fast shades on the fiber, which process consists in treating textile fabrics dyed with sulfurized dyestuffs with neutral sulfites, substantially as hereinbefore described.

In testimony whereof I have signed my name in the presence of two subscribing witnesses.

OSCAR JAECK.

Witnesses:

OTTO KÖNIG,  
EMIL PLUMBERG.